

FIP8309 XR 1,404,242  
CATION OF TEXTILES & FIBERS,

111

## UNITED STATES PATENT OFFICE.

HARRY B. SMITH, OF ALBANY, NEW YORK.

## PROCESS OF BLEACHING MATERIAL.

1,404,242.

Specification of Letters Patent. Patented Jan. 24, 1922.

No Drawing.

Application filed July 19, 1921. Serial No. 485,983.

To all whom it may concern:

Be it known that I, HARRY B. SMITH, a citizen of the United States, and a resident of Albany, in the county of Albany and State of New York, have invented certain new and useful Improvements in Processes of Bleaching Material, of which the following is a specification.

My invention relates to a process of 10 bleaching cotton and other material.

One of the objects of the invention is to provide an improved process of bleaching such material, which is simple, efficient and requires only a relatively short time.

15 The kind of material to which this process is primarily adapted is unbleached cotton goods containing motes, shives and (or) leaf. The process is applicable, however, to any material containing vegetable or animal 20 fibre, such as any class of cotton goods or yarns, wool, silk, fibre silk or mixtures of same.

The process herein disclosed is more 25 economical and efficient than processes heretofore used because the removal of the motes, shives and (or) leaf, the bleaching by an oxidizing agent and the bluing are effected more or less at the same time. In

30 United States Patent No. 1,199,745, to Irwin J. Smith and myself, there is disclosed a process of dyeing in which increased economy is effected by removing the motes, shives and (or) leaf by an oxidizing bath which is markedly alkaline, to which bath a

35 dye is added while the material is still in the solution. In the process of the said patent, however, any tendency to bleach is only incidental, the whole process being carried out solely from the standpoint of removing the

40 motes, shives and (or) leaf without injury to the material and dyeing the same, and the reagents and their strength are chosen accordingly. The process herein described and claimed is primarily to obtain a clean, 45 white, bleached material.

Other objects, features and advantages of my invention will appear more fully in the following detailed description and appended claims.

50 In accordance with my invention, I employ an alkaline oxidizing agent which is preferably composed of about half each of peroxide of sodium and a salt of an alkali metal, such as sodium chloride, soda ash, 55 silicate of soda, caustic soda, phosphate of

soda, alone, or a mixture of any of these salts. The combined weight of the peroxide of sodium and salt of an alkali metal is preferably about seven per cent of the weight of the cotton material under treatment. A solution of these chemicals is 60 strongly alkaline and at the same time oxidizing. Because it is strongly alkaline the time required for removing the motes, shives and (or) leaf is relatively short. At the 65 same time the alkalinity is not sufficiently intense to harden the material to be bleached. This solution has been found to operate with entire satisfaction, but it is understood that any oxygen liberating product, but preferably those corresponding to 70 the "per" salts and preferably for a purpose hereinbefore stated, along with the salt of an alkali metal will give satisfactory results. For instance, peroxide of hydrogen, 75 percarbonate of sodium, persulphate of sodium, or persilicate of sodium, may be used with a suitable salt of an alkali metal or a mixture of salts such as those mentioned above. I have, however, obtained the best 80 results with peroxide of sodium.

The dyes preferably used for bluing are alkali blues, inasmuch as they are substantially operatively unaffected by the oxygen yielding compounds and alkalis which are 85 used in the process. I have, for example, employed in practice as a suitable dye that having the trade name "Alkali Blue R. S.". These dyes and their chemical composition are well known in the art. They are acid 90 dyes, that is, they require an acid to render them effective. Such dyes cause a very brilliant whiteness in the bleached material. While various acids might be used for this purpose, I preferably use an organic acid, 95 such as acetic acid. Such an acid does not attack the fibre of the cotton and gives very satisfactory results in bluing. Furthermore, by its reaction with the sodium peroxide or its equivalent, it liberates oxygen 100 while the bath is at a high temperature, which greatly assists the bleaching operation. At the same time it destroys the organic coloring matter in the cotton, thereby increasing the whiteness of the material. 105

I have found it preferable in my practice of the invention to pursue a detailed procedure substantially as follows, but I do not limit my invention to this exact mode of procedure as it may be varied without departing 110

111  
2

1,404,242

from the invention as set forth in the appended claims: The goods are first washed with boiling water, as is usual in the art, to remove greasy or waxy foreign matter from the fibers. The cotton material is then passed into a bath at normal atmospheric temperature containing the alkali blue. About fifty grains of the dye may be used to one hundred pounds of the cotton material. This bath is allowed to work on the material for about fifteen minutes. The acetic acid is then added to the same bath to develop the color. The acetic acid may be in amount about two per cent of the weight of the cotton material. After the acetic acid has been added, the bath is allowed to act upon the material about ten minutes longer, after which the bath is brought to a high temperature, preferably between 170° and 20 180° Fahrenheit. It is unnecessary to bring the bath to a boil and preferable not to do so. Sodium peroxide and sodium chloride or other alkali metal salt, in the amounts previously mentioned, are now added and 25 the bath maintained hot, preferably between 170° and 180° F., for a considerable period of time. An hour and a half is ample for this last step. It is the function of the sodium chloride or other alkali metal salt 30 to aid in the development and fixation of the coloring matter on the fibre, as well understood in the art.

During the process, the motes, shives and (or) leaf are subjected to a chemical action 35 which probably softens and dissolves them.

It is to be understood that the chemicals, including the bluing, the acid and the proportions of the chemicals and periods of time set forth above, are given as merely examples and that I am not limited to the 40 same.

Having described my invention, what I claim as new and desire to secure by Letters Patent is as follows:

1. The process of bleaching material which comprises subjecting the material to a bath having added thereto an alkali blue, an organic acid, and an alkaline oxidizing agent.

2. The process of bleaching cotton material containing foreign matter which comprises bluing the material with an acid dye and subjecting the material to an alkaline oxidizing bath.

3. The process of bleaching cotton material containing foreign matter which comprises subjecting the material to a hot bath having added thereto an alkali blue, an organic acid, and an alkaline oxidizing agent.

4. The process of bleaching cotton material containing foreign matter which comprises subjecting the material to a bath heated to a high temperature below the boiling point and having added thereto an alkali blue, an organic acid, and an alkaline oxidizing agent.

5. The process of bleaching cotton material containing foreign matter which comprises subjecting the material to a bath heated to a temperature above 170° F. and below the boiling point and having added thereto 70 an alkali blue, an organic acid, and an alkaline oxidizing agent.

6. The process of bleaching material which comprises subjecting the material to a hot bath having added thereto an alkali blue, 75 acetic acid, and an alkaline oxidizing agent.

7. The process of bleaching cotton material containing motes, shives and (or) leaf which comprises treating the material in a bath having added thereto an acid bluing, an 80 organic acid, and an alkaline oxidizing agent adapted to soften or loosen the motes, shives and (or) leaf in said bath, the bluing being substantially operatively unaffected by said alkaline oxidizing agent.

8. The process of bleaching cotton material containing motes, shives and (or) leaf which comprises treating the material in a bath containing an acid bluing, and an organic acid, heating the same, adding to 90 the bath while the material is therein an alkaline oxidizing agent adapted to soften or loosen the motes, shives and (or) leaf in said bath, the bluing being substantially operatively unaffected by said alkaline oxidizing agent, and maintaining the bath heated until the motes, shives and (or) leaf are substantially removed from the material.

9. The process of bleaching cotton material containing motes, shives and (or) leaf which comprises treating the material in a bath containing an acid bluing and an organic acid, heating the same to a temperature over 170° F. and below the boiling 100 point, adding to the bath while the material is therein an alkaline oxidizing agent adapted to soften or loosen the motes, shives and (or) leaf in said bath, the bluing being substantially operatively unaffected by 105 said alkaline oxidizing agent, and maintaining the bath heated at approximately the above temperature until the motes, shives and (or) leaf are substantially removed from the material.

10. The process of bleaching cotton material containing motes, shives and (or) leaf which comprises treating the material in a bath containing an alkali blue, then adding acetic acid, then heating the bath without 110 bringing the same to a boil, then adding sodium peroxide and sodium chloride, and maintaining the bath with the material therein at approximately the above temperature until the motes, shives and (or) leaf 115 are substantially removed from the material.

11. The process of bleaching material which comprises treating the material in a bath containing an alkali blue, then adding 120

acetic acid, then heating the bath, then adding sodium peroxide and sodium chloride, and adding further heat to the bath with the material therein.

- 5 12. The process of bleaching cotton material containing motes, shives and (or) leaf which comprises treating the material in a bath containing an alkali blue, then adding an organic acid, then heating the 10 bath, then adding sodium peroxide and sodium chloride, and maintaining the bath with the material therein heated until the motes, shives and (or) leaf are substantially removed from the material.
- 15 13. The process of bleaching cotton material containing motes, shives and (or) leaf which comprises treating the material in a bath containing an alkali blue, then adding an organic acid, then heating the 20 bath, then adding sodium peroxide and an alkali metal salt, and maintaining the bath with the material therein heated until the

25 motes, shives and (or) leaf are substantially removed from the material.

14. The process of bleaching cotton material containing motes, shives and (or) leaf which comprises treating the material in a bath containing an alkali blue, then adding an organic acid, then heating the bath, then adding an oxygen producing agent and sodium chloride, and maintaining the bath with the material therein heated until the 30 motes, shives and (or) leaf are substantially removed from the material.

35 15. The process of bleaching cotton material containing foreign matter which comprises subjecting the cotton to a bath containing a alkali blue, an organic acid, and an amount of sodium peroxide and sodium chloride equal to approximately 7% of the 40 weight of the cotton material.

In testimony whereof, I have signed my name to this specification.

HARRY B. SMITH.